

## UNITED STATES PATENT OFFICE.

STANLEY D. SHIPLEY, OF STAMFORD, CONNECTICUT, ASSIGNOR TO ATLAS POWDER COMPANY, OF WILMINGTON, DELAWARE, A CORPORATION OF DELAWARE.

## BRUSHING LACQUERS.

No Drawing.

Application filed September 28, 1925. Serial No. 59,164.

This invention relates to nitrocellulose lacquers and lacquer enamels and it has for its object to provide an improved substance of this character of such composition that it can be successfully applied with a brush over previously applied coats of paint, varnish or nitrocellulose lacquer or lacquer enamel, without attacking such previously applied coats.

As far as I am aware, it has not been possible, prior to this invention, to apply a nitrocellulose lacquer or lacquer enamel upon previously coated surfaces of the character indicated, nor has it been possible to successfully apply such lacquer and lacquer enamel with a brush and get a smooth finish free of brush marks.

The reason that it has not been possible to successfully apply these nitrocellulose lacquers and lacquer enamels with a brush, even upon new surfaces, is that the solvents commonly employed, dry or evaporate with such rapidity that "pulling" develops before the brushing can be completed, with the result that brush marks are left and a smooth surface cannot be secured.

Where an attempt has been made to apply a lacquer or lacquer enamel, consisting of a nitrocellulose base, and the commonly known solvents, upon old work, that is, upon surfaces which have been previously coated with paint, varnish or nitrocellulose lacquer or lacquer enamel, the solvent content of the newly applied coat has attacked and softened the undercoating and it has not been possible to get a good finish. This is particularly true if the application of the newly applied coat is with a brush, where the mechanical action of the brush tends to dislodge and slough off the softened undercoatings.

To avoid the foregoing difficulties and to produce a nitrocellulose lacquer or lacquer enamel which may be successfully applied by brushing, either upon new work or over previously applied coatings, I reduce the amount of active solvent in the lacquer to a quantity just sufficient to keep the nitrocellulose in solution and I employ, in conjunction therewith, a substantial proportion of a diluent consisting of a petroleum hydrocarbon, such as gasoline.

Furthermore, I employ a solvent having markedly slower drying qualities than the solvents commonly employed in nitrocellulose lacquers, such as amyl acetate, acetone, butyl acetate, etc. In addition, the rates of evapo-

ration of the solvent and the petroleum hydrocarbon diluent employed, are such as to insure the evaporation of the diluent ahead of the complete evaporation of the solvent, since otherwise the nitrocotton would be precipitated from the solution and the nitrocellulose film would be spoiled. It would be hazy, very weak and probably non-adherent.

By extensive experimentation I have found ethylene glycol mono ethyl ether



hereinafter referred to as ethyl glycol, to be particularly adapted for use in the relation set forth, because its rate of evaporation is so slow that the product may be applied with a brush and brought to a properly smoothed finish before the drying has proceeded to such a point as to prevent brushing. Furthermore, the rate of evaporation of the ethyl glycol, with respect to the rate of evaporation of the gasoline, is such as to insure the dissipation of all of the latter ahead of the removal of the former, so that the possibility of precipitation of the nitrocellulose is eliminated.

An additional advantage inherent in the product of the present invention is the absence of the highly objectionable odors common to the ordinarily employed solvents if nitrocellulose such as amyl acetate, for example.

In the manufacture of nitrocellulose lacquers, it is common to dissolve a base of nitrocellulose and glycerine resin ester (a resin) in a suitable solvent or mixture of solvents or, and, diluents and if a lacquer is desired, suitable pigments are added to the otherwise clear lacquer. I employ to advantage the following formula.

An example of a brushing enamel (a pigmented lacquer) is—

|              | Per cent.          |
|--------------|--------------------|
| Ethyl glycol | 40                 |
| Gum solution | 25                 |
| Gasoline     | 35                 |
|              | 100                |
| Nitrocotton  | 12 oz. per gal.    |
| Titanox      | 3.25 lbs. per gal. |

The gum solution is a six pound cut of gum in toluol.

The proportion of gasoline and ethyl glycol will vary with the kind and amount of gum solution used, the presence or absence of other nitrocotton solvents, and the kind and quan-

tity of other non-solvents for nitrocotton which may be present.

It is not to be understood that the diluent used must consist wholly of gasoline or other petroleum hydrocarbon. Other diluents may be present. It is only necessary that a substantial proportion of the diluent be a petroleum hydrocarbon of the nature of gasoline which, experience has shown, has no such destructive effect upon previously applied coatings as most of the commonly used diluents, such as toluol or benzene, for example. I am aware of the fact that it is common practice to use gasoline as a diluent in nitrocellulose solvent compositions. However, to the best of my knowledge and belief, gasoline has never been designedly employed with a slow drying solvent to make a brushing lacquer, nor with a solvent wherein the rates of evaporation of the solvent and diluent were in determined relation, to the end of producing a lacquer which could be applied by brushing and yet give a smooth finish, and which would not attack undercoats, either through the action of the solvent or the action of the diluent.

While I prefer to use ethyl glycol as my slow drying solvent, I may mention as other practicable slow drying solvents, methyl and ethyl benzoate, methyl salicylate, ethyl lactate, ethyl oxalate, adronal acetate, etc. All of the above solvents mix well with gasoline. By a "slow drying" solvent as defined in the appended claims, I mean a solvent drying slower than amyl acetate. Since ethyl glycol is a much more active solvent for nitrocellulose than many of the commonly used solvents, such as ethyl, butyl and amyl acetate, for example, a much smaller percentage of ethyl glycol will serve to keep the nitrocellulose in solution and a much greater quantity of diluent, such as gasoline, may be used.

Since practically all undercoatings contain resins, it follows that diluents which are solvents of resins are destructive of undercoatings. Benzene, toluene, xylene, etc., are much more powerful solvents of practically all of the resins, such as copal, shellac, sandarac, demar, kauri, Pontianak, etc., than gasoline. Gasoline has little, if any, solvent effect upon these resins.

Having described my invention, what I claim is:

1. A brushing lacquer including a nitrocellulose base, ethyl glycol as a solvent and gasoline as a diluent wherein the gasoline is in

such proportions that when the lacquer is applied in a finishing coat the ethyl glycol while maintaining the nitrocellulose in solution without precipitation, will not appreciably attack previously applied coats of lacquer, paint or varnish. 60

2. A liquid vehicle for nitrocellulose lacquers, the major portion of which consists of a slow drying solvent and gasoline and wherein the amount of gasoline is within ten percent 65 of the amount of the slow drying solvent.

3. A brushing lacquer consisting in the main of a nitrocellulose base, ethyl glycol as a solvent and gasoline as a diluent, the proportions of the ethyl glycol and gasoline being such that the solvent barely maintains the nitrocellulose in solution and does not exercise any appreciable effect upon previously applied undercoatings, the gasoline evaporating ahead of the ethyl glycol, whereby precipitation of the nitrocellulose is prevented. 70 75

4. A brushing lacquer comprising a nitrocellulose base, a slow drying solvent and gasoline, the proportion of the solvent and gasoline being such that when the lacquer is exposed to the air by being applied in a brushing coat, the gasoline will be removed by evaporation ahead of the solvent whereby precipitation of the nitrocellulose is prevented. 80 85

5. A brushing lacquer consisting in the main of a nitrocellulose base, ethyl glycol as a solvent and gasoline as a diluent, the gasoline constituting substantially 35% of the liquid content of the lacquer, and the proportion 90 of gasoline and solvent being such that the solvent barely maintains the nitrocellulose in solution and does not exercise any appreciable softening effect upon previously applied undercoatings, the gasoline evaporating ahead 95 of the ethyl glycol whereby precipitation of the nitrocellulose is prevented.

6. A nitrocellulose brushing lacquer, consisting of a nitrocotton base, and a liquid vehicle comprising the following ingredients 100 combined in substantially the proportions stated

|              | Per cent. |
|--------------|-----------|
| Ethyl glycol | 40        |
| Gum solution | 25        |
| Gasoline     | 35        |

In testimony whereof he affixes his signature.

STANLEY D. SHIPLEY.